

## UNITED STATES PATENT OFFICE.

FRANK H. BERGEIM, OF WOODBURY, NEW JERSEY, ASSIGNOR TO E. I. DU PONT DE NEMOURS & COMPANY, OF WILMINGTON, DELAWARE, A CORPORATION OF DELAWARE.

## CYANO NITRATE EXPLOSIVE AND PROCESS OF PRODUCING THE SAME.

No Drawing.

Application filed September 15, 1927. Serial No. 219,817.

This invention relates to explosives containing one or more cyano groups and one or more nitrate groups. It relates particularly to explosives comprising a hydrocarbon which 5 has attached thereto cyano groups and nitrate groups, and also relates to the process of producing said explosives.

One object of the invention is to provide a new type of explosive of the above character combining in part the explosive groupings of nitroglycerine and hydrocyanic acid.

Another and more particular object is to provide an explosive of this type in which one or more cyano ( $-\text{CN}$ ) groups and one or more nitrate ( $-\text{ONO}_2$ ) groups are attached 15 to a hydrocarbon.

A further object of the invention is to provide a product which may be used alone or in combination with the usual dynamite 20 ingredients to make a dynamite of good strength and great insensitiveness to mechanical shock.

The product cyano methanol nitrate,  $\text{CNCH}_2\text{ONO}_2$ , has previously been prepared, 25 but by an expensive method involving the use of silver nitrate and potassium iodide, which is impractical from the viewpoint of economy. Accordingly, a still further object of my invention is to provide a novel, practical and 30 relatively inexpensive process for producing this and other products.

By the process of my invention, which has a wide application, a cyanohydrin is nitrated with mixed acid to give a cyano nitrate explosive. The above mentioned explosive, 35 cyano methanol nitrate, may thus be made by the nitration of methylene cyanohydrin,  $\text{CNCH}_2\text{OH}$ .

Further objects and advantages of the invention will appear from the following description and detailed examples of the invention.

Cyano nitrate explosives in which the cyano and nitrate groups are attached to the same 45 carbon atom are acidic in character and relatively unstable. I have found that cyano nitrate explosives having the cyano and nitrate groups on different carbon atoms, in

accordance with the present invention, as for example cyano ethanol nitrate, 50



possess an unusually good stability. Another example of this type of explosive is that formed by the nitration of the cyanohydrin 55 of glycerine,



which gives cyano propanediol dinitrate,



The cyano nitrate explosives having the cyano and nitrate groups each on different carbon atoms may be made in any desired way. I prefer, however, to make them by 65 treating cyanohydrins with mixed acid. One example of the way in which my process may be carried out is the following.

If the case of cyano ethanol nitrate, I may add one part by weight of cyano ethanol, 70 prepared in any desired way, to two and one-half parts by weight of mixed acid comprising approximately 40% nitric acid and 60% sulphuric acid either in the absence of water or with not more than 10% water present, 75 the temperature being kept between 0° and 10° C. The high solubility of the nitrated product in the waste acid necessitates drowning to obtain the explosive oil. This oil may then be neutralized by washing with a weakly 80 alkaline solution such as a 5% solution of sodium carbonate. The product thus obtained is a neutral, colorless oil of about the same viscosity as glycol dinitrate. It has been found to retain its neutrality over a period of 85 several months storage. Analyzed for nitrate nitrogen by the nitrometer method, it gave a value very near to the theoretical (12.07%). This oil, while not quite as powerful as ethylene glycol dinitrate, has the desirable property of being much less sensitive to mechanical shock than the latter.

Cyano ethanol nitrate may be used alone as an explosive or in combination with the usual dynamite ingredients to make a dynamite of good strength and great insensi-

tiveness to mechanical shock. It may be used in a dynamite comprising nitroglycerine or its substitutes, as, for example, mixtures of nitroglycerine with tetranitrodiglycerine, 5 nitro sugars, or nitroglycol. The following composition may be cited as a specific example of a dynamite in which the new explosive may be used:

|                          | Parts<br>by weight. |
|--------------------------|---------------------|
| 10 Cyano ethanol nitrate | 15                  |
| Glycerine trinitrate     | 15                  |
| Sodium nitrate           | 58                  |
| Wood meal                | 11                  |
| 15 Chalk                 | 1                   |

In addition to its use in non-gelatinous explosives, of which the above formula is a typical example, the cyano nitrate explosives may be used for the manufacture of gelatinous explosives, in which case it is gelatinized with nitrocellulose.

Furthermore, instead of the sodium nitrate, or in addition thereto, I may use various other oxidizing salts, as, for example, 25 ammonium nitrate, ammonium perchlorate or potassium nitrate. Also, it will be understood that the various known carbonaceous combustibles for use in explosives may be used in connection therewith instead of or together with the wood meal. Also, other mineral fillers may be used instead of or together with the chalk hereinabove referred to.

It is to be understood, however, that in all the above compositions the proportions may 30 vary widely as to each and all of the ingredients, according to the particular uses to which the explosive is to be applied.

While I have described my invention in de-

tail, it is to be understood that many changes may be made in the examples above given 40 without departing from the invention as defined by the following claims.

I claim:

1. An explosive compound containing a cyano group and a nitrate group. 45
2. An explosive compound comprising an aliphatic ester containing a cyano group and a nitrate group.
3. An explosive compound comprising an aliphatic ester containing a cyano group and a nitrate group, said groups being each attached to different carbon atoms therein. 50
4. As a new chemical compound, cyano-ethanol-nitrate.
5. The process which comprises producing 55 a cyano nitrate by the nitration of a cyano alcohol.
6. The process which comprises producing cyano ethanol nitrate by the nitration of cyano ethanol. 60
7. The process which comprises producing a cyano nitrate by nitration of a cyano alcohol and washing the separated product with an alkaline solution.
8. The process which comprises producing cyano ethanol nitrate by the nitration of cyano ethanol and washing the separated product with an alkaline solution. 65
9. The process which comprises producing cyano ethanol nitrate by the nitration of cyano ethanol with mixed acid, and washing the separated product with an alkaline solution. 70

In testimony whereof, I affix my signature.

FRANK H. BERGEIM.